

May 14, 1935.

J. R. FORDYCE

2,001,130

REVESTMENT

Filed Dec. 3, 1932



Inventor:  
JOHN R. FORDYCE,

*John H. Bunninga*  
His Attorney.

## UNITED STATES PATENT OFFICE

2,001,130

## REVETMENT

John R. Fordyce, Hot Springs, Ark.

Application December 3, 1932, Serial No. 646,471

4 Claims. (Cl. 61—38)

This invention relates generally to the protection of revetments such, for instance, as levees, river banks, canals and irrigation ditches, and particularly to revetment mats and the method of making and applying the same to the revetment.

In the protection of revetments, it has heretofore been the practice to launch and suitably secure to the banks, mats which may be formed of bundles of willows woven together as by means of wire cables. Some attempts have been made to provide a series of concrete slabs suitably secured together so as to provide a revetment mat and it has also been attempted to provide such mats in which a permanently flexible binder as, for instance, asphalt oil is used in compositions with stone, sand and the like, and provided with suitable re-enforcements to form revetment mats. Mats wherein asphaltic oils and similar materials are employed, so as to render the mat permanently flexible, are, however, of relatively short life due to the fact that the asphaltic oil or other fluid binder is readily scoured out of the composition by the current of the stream and by the sand which is carried by it so that such mats are of extremely short effective life.

The object of the present invention, generally stated, is to provide a revetment mat which will readily conform itself to the contour of the revetment or stream bank upon being launched, but which is of such character as to resist the erosive action of the water.

A further object of this invention is to provide a revetment mat and a method of applying the same whereby the mat, although soft when launched, will harden upon exposure to the water so as to form a hard and resistant protection to the stream bank.

A more specific object of this invention is to provide a revetment mat wherein the binder employed is one which is at ordinary temperatures hard and resistant, but which may be softened upon heating so as to be workable.

Other objects will become apparent to those skilled in the art when the following description is read in connection with the accompanying drawing which illustrates in detail a section of revetment mat constructed in accordance with this invention.

In accordance with the present invention generally stated, a suitable water proofing binder material such, for instance, as an asphaltic substance which is hard and resistant under ordinary conditions but which may be softened for working may have incorporated with it a suitable quan-

tity of mineral aggregate such, for instance, as gravel, sand, broken stone of silicious, argillaceous or calcareous nature, or if desired, of a class of heavy mineral substances such, for instance, as barite or hematite. The aggregate should, of course, be so selected as to size as to produce a matrix having a maximum specific gravity and a low percentage of voids. In the matrix resulting from the mixture of asphaltic substance and mineral aggregate as just described, may be embedded a series of suitable metallic re-enforcements which may be in the form of wire mesh, interwoven cables, expanded metal or other suitable re-enforcements, preferably flexible. In accordance with the present invention, the asphaltic substance which at ordinary temperatures is normally hard, may be heated to a temperature substantially above its softening point so as to render the same workable and while maintained at this temperature may be incorporated with the aggregate and have the metallic re-enforcements embedded in it. Furthermore before the temperature of the asphaltic substance drops below the softening point, the resultant re-enforced mat is, in accordance with the present invention, launched into the stream and secured to the revetment. In this manner advantage is taken of the flexibility of the asphaltum while at the elevated temperatures so that the mat may conform itself to the contour of the revetment, but upon exposure to the water it will be understood that the asphaltum will cool below its softening point so as to present a hard resistant mat which will efficiently protect the banks of the stream and be of substantial life.

As a specific illustration of a practical embodiment of the invention, the binder material selected may be asphaltum which is hard at ordinary temperatures and little affected by water or climatic temperature changes, but which may be softened at about 150° F. A suitable quantity of such asphaltum, for instance, sufficient to comprise 20% of the matrix to be formed may be heated to a workable temperature as, for instance, about 350° F.

A suitable quantity of mineral aggregate, for instance, sufficient to comprise about 80% of the matrix to be formed, may, after being carefully graded and washed, be heated to a temperature approaching the working temperature of the asphaltum as, for instance 300° F. When the mineral aggregate is heated to this extent, it will be understood that the same may be incorporated with the asphaltum without cooling the latter to an extent such that it will become unworkable.

On a platform or other flat surface of suitable size the asphaltum aggregate mixture may be formed into sheets or slabs while the asphaltum is maintained at a working temperature. The platform may be dusted over with limestone dust, talc or Portland cement in order to prevent the asphaltum from sticking thereto. Across the platform the metallic re-enforcements, which may be in the form of a metallic mesh or fabric, may be spread and on to this the desired quantity of the asphaltum aggregate mixture, after being thoroughly incorporated, as in a pug mill, may be spread. Enough of the asphaltum aggregate mixture may be spread to form a sheet or slab of the desired thickness and the mixture may then be compacted about the re-enforcements, as by tamping or rolling to an extent sufficient that the mixture entirely surrounds and encloses the re-enforcements so as to form a water proof coherent mass. It will be understood that during all these operations the temperature of the asphaltum aggregate mixture is maintained above the softening point for the asphaltum and preferably sufficiently high that the asphaltum may completely coat the metallic reenforcement so as to protect the same from corrosion.

Before the sheet or slab thus formed has cooled below the softening point for the asphaltum and preferably while the same is at a temperature considerably above that point, the sheet or slab may be launched or applied to the revetment or stream bank. In accordance with the present invention the temperature of the slab or sheet is preferably at this time sufficiently above the softening temperature for the asphaltum that the slab or sheet may sink into position beneath the water and conform itself to the contour of the revetment or stream bank before hardening.

When the aggregate employed is of a heavy mineral such, for instance, as a class including barite and hematite, it is apparent that the sheets or slabs formed in accordance with the present invention may be caused to sink beneath the surface of the water without the use of extraneous means, the specific gravity of the mineral being sufficient to sink it and maintain the same against displacement by the stream current. It will be understood, of course, that the mats may be formed of lighter minerals and the sheets or slabs suitably anchored or otherwise secured to the stream banks to prevent displacement.

It will be understood that the amount of asphaltum may be varied in accordance with the requirements of a particular stream and the size of the aggregate employed, as from 5% to 25% by weight of the mat. The thickness of the mat may be varied from one-half to six inches, depending upon stream conditions and the character of materials employed. As pointed out hereinbefore, a sufficient quantity of asphaltum is preferably employed to completely coat the metallic re-enforcement so as to protect the same from corrosion and, if desired, the wire mesh or other metallic re-enforcement may be given a pre-coat of asphaltum.

It will be understood that the metallic re-enforcement employed may be of any suitable character, preferably of sufficient flexibility to permit the mat to adapt itself to the contour of the revetment or stream bank.

From the foregoing description it is apparent that the present invention contemplates a method of protecting revetments wherein the mat employed is of such composition as to effectively resist the erosive action of the sand carried by a stream and that the revetment mat of the present invention, although sufficiently pliable to conform itself to the contour of the stream bank at the time of launching, will immediately become sufficiently hard to be resistant. It is apparent that many modifications of the revetment mat and the process of making and applying the same hereinbefore described will occur to those skilled in the art which will not depart from the spirit of this invention. It is to be distinctly understood, therefore, that the invention is not limited to the specific details hereinbefore described for the purpose of illustration, but that such modifications and the use of such individual features and sub-combinations of features as do not depart from the spirit of this invention are, although not specifically described herein, contemplated by and within the scope of the appended claims.

Having thus described the invention, what is claimed is:

1. In the art of protecting revetments, the process comprising, heating normally hard asphaltum to a temperature substantially above its softening point, mixing mineral aggregate with the asphaltum, working the hot asphaltum-aggregate mixture about a substantially flat reenforcing network to form a self-sustaining sheet, and launching the sheet before the mixture cools to below the hardening temperature.

2. In the art of protecting revetments, the process comprising, heating normally hard asphaltum to a temperature of about 350° F., pre-heating a mineral aggregate to a temperature of about 300° F., incorporating the hot asphaltum and aggregate, working the hot mixture around a reenforcing network to form a self-sustaining sheet, and launching the sheet.

3. A revetment mat comprising a matrix of a mineral aggregate in a binder of normally hard asphalt which is resistant to water and erosion, and a reinforcing structure embedded in and completely enclosed by said matrix, said reinforced matrix being in the form of self-sustaining sheets.

4. A revetment mat comprising a self-sustaining sheet preformed so as to be launched upon the bank of a stream, said mat composed of a metallic reinforcement imbedded in and completely enclosed by a matrix of normally hard asphalt and mineral aggregate, the asphalt being of such character as to form a permanently hard surface at atmospheric temperatures.

JOHN R. FORDYCE.

65